

No. 881,221.

PATENTED MAR. 10, 1908.

A. BONTEMPI.

RUST PROOFING IRON, STEEL, &c.

APPLICATION FILED JAN. 29, 1907. RENEWED JAN. 28, 1908.



INVENTOR

Augusto Bontempi,

By Attorneys,

Arthur C. Racine & Urena

WITNESSES:

Fred Whits

René Prune

# UNITED STATES PATENT OFFICE.

AUGUSTO BONTEMPI, OF NEW YORK, N. Y.

RUST-PROOFING IRON, STEEL, &c.

No. 881,221.

Specification of Letters Patent. Patented March 10, 1908.

Application filed January 29, 1907, Serial No. 354,672. Renewed January 28, 1908. Serial No. 412,991.

*To all whom it may concern:*

Be it known that I, AUGUSTO BONTEMPI, a subject of the King of Italy, residing in the borough of Manhattan, city, county, and

5 State of New York, have invented certain new and useful Improvements in Rust-Proofing Iron, Steel, or the Like, of which the following is a specification.

The object of the invention is to produce a 10 surface which prevents rusting even under severe conditions such as subjection to high temperature and corrosive influence, water, salt water, etc.

15 The invention provides certain improvements over the method described in my prior application No. 285,240 dated October 31, 1905 and adapted also for use in connection with the process of said application.

The desired effect is obtained by heating 20 the iron to approximately from 1000 degrees F. to 1800 degrees F. in a closed and preferably airtight chamber, the iron having been previously treated according to the Bower-Barff process or not as desired, and 25 subjecting it to the gas or vapor of one or more non-corrodible substances. Where the Bower-Barff treatment is omitted the temperature need be only high enough to insure volatilization of the non-corrodible substance. For example for zinc, lead and other volatile non-corrodible metals the temperature will generally be within 1000 degrees F. At the time of applying the gases the metal under treatment will be very much expanded 30 by the heat and the pores, especially those at the surface will be opened to receive the gases which will penetrate to a considerable depth depending upon the period of time and other conditions. When the metal cools 35 after the treatment, the vapors are first reduced to a solid condition, and by the further cooling of the metal a very dense and substantially non-corrodible surface is produced.

40 45 Wherever heavy goods are being treated they will usually be subjected to the Bower-Barff process first. But for light flexible goods the Bower-Barff process may be omitted, the resulting coating being less brittle 50 by reason of the omission.

Where the goods are first subjected to steam according to the Bower-Barff process, lime or some equivalent alkaline material may be introduced serving to insure a perfect dryness of the steam and particularly 55 also facilitating the formation of the coating

by a catalytic action. I may also inject with the steam a small quantity of naphtha or other hydrocarbon which gives a desirable black color to the coating.

60

The goods under treatment are preferably carried in a closed metal chamber with a surrounding chamber of fire brick. Where the goods are not intended for the hardest use, however, the goods need not be carried 65 in a perfectly airtight chamber but may be in an open pan within the chamber of fire brick which is comparatively tight.

A suitable apparatus for carrying out the process is illustrated diagrammatically in the 70 drawings.

Referring to the drawings, A is the boiler furnishing the desired steam, which passes by a pipe B to a coil C running back and therefore in the chamber D of fire brick and arranged on three sides of the sheet iron or steel muffler or chamber E in which the goods to be treated, such as the pipe F, are carried. A fire box G is arranged below the chamber D, the products of combustion being carried 75 by any suitable arrangement of flues about the muffler E so as to maintain the latter at the desired temperature.

A tray of lime H may be introduced into the muffler before the latter is closed and 80 heated. A branch J permits the injection of naphtha into the steam.

Any suitable means such as the pipe K may be used for introducing the non-corrodible materials after the goods are heated to 85 the desired high temperature.

Where treatment by steam is not to be used in any particular case, of course, it will not be necessary to use anything more than the muffler with means for heating it and for 90 introducing the non-corrodible materials. Supposing, however, that the process is to comprise all the various steps described, the operation is as follows:—The goods are filled into the muffler which is placed in the fire 95 brick chamber and the latter substantially sealed after making the several connections. The muffler and contents are heated to from 1000 to 1800 degrees Fahrenheit approximately and then the steam from the boiler 100 A is introduced and the process continued until the usual black oxid is produced to the desired depth. Thereupon, while maintaining the temperature of the muffler, the steam is cut off and the non-corrodible material introduced.

As examples of the non-corrodible mate-

rial, I may use (1) tannic acid, an oleaginous material, and a non-corrodible metal such as zinc or an oxid of such metal; or (2) a pure metal such as zinc or lead; or (3) substantially solid hydrocarbons such as coal tar or pitch. The first of these compositions gives a good coating of dark gray color, the second gives also a good coating of blue color, but the third gives a black coating of the very highest quality. I have tested goods made with this black coating under all known conditions for rusting and have found them to be perfectly rust proof under all tests.

Of the three non-corrodible materials above described the best results are obtained by treatment first with the non-corrodible metal (either alone or in the combination with tannic acid and oleaginous material) and then with the hydrocarbon.

20 The process will be continued from 2 to 6 hours according to the depth of treatment desired and the weight of the goods, having regard to the weakening of the fiber which might be serious in light goods.

25 Before the treatment the metal is washed perfectly clean as usual in rust proofing processes. After the goods are taken out of the retort they are cooled to about 100 degrees F. and greased with vaseline and cleaned so as 30 to give them a good polish and of attractive appearance.

Although I have described with great particularity of detail certain specific embodiments of my invention, yet it is not to be understood therefrom that the invention is restricted to the particular embodiments disclosed, as various modifications thereof in detail may be made by those skilled in the art without departure from the invention.

What I claim is:—

1. The method of protecting iron or steel which consists in subjecting it to the Bower-Barff treatment and subsequently subjecting it to the vapor or gas of a non-corrodible metal substance while heating it to a high 45 temperature in a closed chamber.

2. The method of protecting iron or steel which consists in subjecting it to the Bower-Barff treatment, and then subjecting it to the vapor or gas of a non-corrodible metal 50 substance while heated in a closed chamber, and finally subjecting it to the vapor or gas of a hydrocarbon while heated in a closed chamber, the temperatures in such closed chambers being in each case sufficiently high to 55 form the vapor or gas referred to.

3. The method of protecting iron or steel which consists in subjecting it in a closed chamber at a temperature sufficient to form such a vapor or gas, to the vapor or gas of a 60 composition including tannic acid, an oleaginous material, and an oxid of a non-corrodible metal.

4. The method of protecting iron or steel which consists in subjecting it in a closed 65 chamber at a temperature sufficient to form such a vapor or gas, to the vapor or gas of a composition including tannic acid, an oleaginous material, and an oxid of a non-corrodible metal, and following this by similar treatment with a solid hydrocarbon.

In witness whereof, I have hereunto signed my name in the presence of two subscribing witnesses.

AUGUSTO BONTEMPI.

Witnesses:

DOMINGO A. USINA,  
FRED WHITE